

## UNITED STATES PATENT OFFICE

2,339,213

COLOR DEVELOPMENT PROCESS USING  
AROMATIC HYDRAZINES

David W. Woodward and David M. McQueen,  
Wilmington, Del., assignors, by mesne assignments,  
to E. I. du Pont de Nemours & Company,  
Wilmington, Del., a corporation of Delaware

No Drawing. Application October 16, 1939,  
Serial No. 299,760

18 Claims. (Cl. 95—88)

This invention relates to photography and more particularly to color photography, and still more particularly to color development processes for photographic elements. In a more limited sense it relates to the production of dye images in photographic elements utilizing aromatic hydrazines as developing agents.

This invention has for an object the production of photographic images in color. A further object is to provide a process for producing color images of improved fastness to light. A still further object is to provide a process for providing stable color images which are not affected by the products produced in the hydrolysis of film base or photographic layers. A still further object is to produce azo dyes during the development of photographic films containing reducible silver salts. A still further object is to provide a new reversal process of developing in which aromatic hydrazines react under conditions of development with a coupling component at the point of the silver salt images to produce azo dyes in situ with metallic silver. Still other objects will appear hereinafter.

One important aspect of the invention involves the treatment of bleached silver images and residual silver salt images. It has been found that the hydrazines are not sufficiently active in many instances to develop exposed or latent images and form dyes with coupling components which are of proper density. It has been found, however, that bleached or reversed images may be effectively reduced with hydrazines and dye images obtained. After the dye images are formed the silver and silver salts are removed with Farmer's reducer or any other suitable bleaching and fixing bath. In the reversal procedures a plurality of reversed images can be simultaneously developed to color component dyed images which result in natural color photographs if the proper emulsions and coupling components are used.

In another important embodiment of the invention developing baths containing mild oxidizing agents and hydrazines are used in the development procedures. It has been found that the coupling velocity and dye density are increased by such procedures.

According to one aspect of the invention, dye coupling components which are soluble in or can readily be dispersed in developer solutions are used in conjunction with aromatic hydrazines. In another aspect of the invention, dye coupling components which are non-migratory and non-leachable from photographic emulsion

layers, e. g. gelatino silver halide emulsion layers, are used. In this latter embodiment of the invention a plurality of emulsion layers sensitized to approximately one third of the visible spectrum is used. Thus, a multilayer film composed of three silver halide emulsion layers which are differentially sensitized are provided with non-migratory azo coupling components which form dyes upon development complementary in color to the sensitivity of the respective layers.

10 In each of the embodiments of the invention, the hydrazine is apparently oxidized during the reduction of the silver images to an intermediate which reacts with a coupling component to form an azo dye.

The mild oxidizing agents may be used with soluble or non-migratory coupling components.

It is well known in the art that phenylhydrazine may be oxidized under certain conditions either to phenol or benzene diazonium chloride by certain inorganic salts (Richter's Organic Chemistry, Vol. II (1929) p. 150). Although the action of silver salts on phenylhydrazine is apparently not known, it is possible that one of these reactions would occur during development of photographic films containing silver salts with aromatic hydrazines.

It has been found that a certain selected group of hydrazines which can be readily ascertained 30 by a simple test give good results and form preferred reducing agents. These hydrazines react with readily reducible silver salts to give intermediates that couple with certain aromatic phenols, amines, and active methylene compounds to give azo dyes. The hydrazines are in 35 general free from negative groups such as sulfonic acid or sulfonate groups and carboxylic acid or carboxylate groups. Suitable hydrazines may be determined by a test as follows:

40 An ammoniacal silver nitrate solution is prepared by dissolving one part of silver nitrate in 200 parts of water and adding concentrated ammonia water until the first formed precipitate has just dissolved. Fifty parts of concentrated ammonia water is then added and the total solution made up to 1000 parts with distilled water. To 10 parts of this solution at 20° C. is added one part of a 1% solution of the aromatic hydrazine to be tested. If during 30 seconds 45 black metallic silver is deposited, the hydrazine is suitable for use in this process, but if there is no silver deposited at this point, the hydrazine is inoperable in this process.

Such hydrazines as selected by the above detailed test may be used as photographic color

developers in alkaline baths of the usual type for they are oxidized directly by the more readily reducible silver salts. However, they are preferably used as stated above with reverse, bleached or non-exposed silver salt images and/or in conjunction with mild oxidizing agents, e. g. hydrogen peroxides, persulfates, hypochlorites, and the like. The intermediate products produced by these treatments apparently readily form coupling diazonium compounds.

These active diazo compounds form azo dyes in the presence of suitable coupling components such as are known in the dye chemistry art (see Fierz-David, *Kunstliche organische Farbstoff*, pp. 87-204). Such coupling components are in general aromatic in nature and possess any one of a number of different substituents such as phenolic hydroxyl, alkoxy, amine, alkylamine and arylamine with replaceable hydrogen atoms or groups in the ortho and/or para position to them, or they may be such reactive methylene groups as are known to enter the coupling reaction. The aromatic hydrazines in such developing solutions are solubilized according to the method described in application Serial No. 299,762 James E. Kirby, filed upon October 16, 1939, entitled Developer solutions now U. S. P. 2,220,929. Suitable solubilizing agents include the water-soluble alkali metal, ammonium and amine salts of stearic, palmitic, oleoic, arachidic, oleostearic, ricinoleic, 12-hydroxystearic, myristic, linoleic acid, the same salts of primary or secondary aliphatic hydrocarbon sulfonic acids containing at least 8 carbon atoms, e. g. of dodecane, tetradecane, octadecane, and 3,10-diethyltridecane-sulfonic acids, mineral oil sulfonates, etc.; the alkali metal, ammonium and amine salts of alkylated aromatic sulfonic acids, e. g. containing a carbon chain of at least 8 carbon atoms, p-dodecylphenolsulfonic, oleo - p-anisidinesulfonic, etc. acids, alkyl sulfates of 8 to 24 carbon atoms, e. g. dodecyl-, tetradecyl, and octadecyl-sulfate, etc., oleyl sulfate, diethyl cyclohexylamine dodecyl-sulfate, etc. As examples of suitable salt-forming groups, mention is made of sodium, potassium, ammonium, alkylolamine, e. g. mono-, di- and tri-ethanolamine, methyl and ethyl amines, etc. Reaction products of long chain carboxylic acids with taurine, isethionic acid, etc. are also useful.

As examples of suitable betaine compounds which may be used are C-(n-hexadecyl- $\alpha$ -)betaine, C-(n-dodecyl)- $\alpha$ -betaine, and the salts of the corresponding open chain betaine compounds. Mixtures of the above agents may be also used. These developing solutions may vary from weakly acid to moderately basic in nature, i. e., from about pH values 6 to 12, depending upon the choice of hydrazine and coupling component. Alkaline solutions, however, are preferred. Solutions of these pH values may be obtained by any of the customary methods used in organic chemistry and they may contain any of the following or closely related types of compounds: weak organic acids such as acetic and the like; salts such as alkaline carbonates, phosphates, acetates, phthalates, citrates, borates and the like, or alkali hydroxides.

There are two procedures which may be used in preparing azo dye images by this process. One consists in adding to the hydrazine developing solution a soluble coupling component which will be converted by the diazo compound pro-

duced on development to an insoluble azo dye at the point of development. To produce a negative image in azo dyes a film bearing a bleached negative silver image is introduced into a developing solution as described above and after development the silver and silver salts are removed by any standard method, e. g., as by Farmer's reducer. To produce a positive or reverse image in azo dyes, the film is exposed and given a preliminary development in a non-color forming developer e. g. "Metol"-hydroquinone. The film is then processed with the hydrazine type of developer as described above. Also, a film containing a positive or negative silver image may be bleached to redevelopable silver salts, as, for example, with potassium ferricyanide, copper chloride or copper bromide in the presence of an oxidizing agent such as chromic acid, potassium ferricyanide in the presence of alkali carbonate or ammonia, etc., and then re-developed in such a color-forming developer as described above. In all cases a film is obtained bearing a clear, bright azo dye image in which the dye has been deposited at the point of reduction of the silver salts and proportional to the amount of silver salt reduced.

Another method for producing films containing azo dye images by this same process as mentioned above, consists in using films in which 30 a nonmigratory coupling component has been incorporated in the emulsion. These are coupling components which, on account of their chemical constitution or molecular size, remain firmly bound in gelatin films and are not leached 35 from them nor migrate in them when the films are placed in the customary baths used in color photography.

The speed of development by the hydrazine solutions may be controlled if desired by the 40 addition of ammonia, which slows the reaction considerably. Thus the addition of about 1% of concentrated ammonia water, for instance, will about double the time of development.

By choice of suitable coupling compounds, it 45 is possible to secure a most complete color range of azo dyes; thus phenols and active methylene compounds will produce yellow to orange dyes. Naphthols will produce colors ranging from red-orange through red to purple, and certain 50 phenylenediamines, aminophenol, and amino-naphthol derivatives will yield colors ranging from blue to blue-green. We are not limited by such classification, however, as these and many other combinations producing azo dyes and 55 well-known in azo dye chemistry (see Fierz-David) are applicable. Nor are we limited to monoazo dyes for by either the use of a difunctional hydrazine as a developing agent or a coupling component containing an azo group or 60 both, it is possible to prepare films containing bis-, tris-, or tetra-kis azo dyes.

The invention will be further illustrated but is not intended to be limited by the following examples, wherein the parts stated are parts by weight:

#### Example I

A photographic film containing a light-sensitive silver halide-gelatin emulsion is exposed and 70 developed in a Metol-hydroquinone developer. The film is then washed, re-exposed to light, and processed in a bath prepared by adding to a mixture of 90 parts of water and 5 parts of 2% sodium oleate, 2 parts of phenyl hydrazine, 2 parts of sodium carbonate and 1 part of sodium beta-

naphtholate, at a temperature of about 8° C., for a period of 10 to 15 minutes. After development the film is thoroughly washed and placed in a 4% solution of potassium ferricyanide for five minutes, washed, and placed in 25% sodium thiosulfate for five minutes, then thoroughly washed. The resulting film contains a clear bright orange azo dye image. The dye has the following probable structure:



Example II

In an experiment similar to that described in Example I and using the sodium salt of acetoacetanilide, prepared by dissolving 1 part of acetoacetanilide in 5 parts of 2% sodium hydroxide solution, a film was obtained bearing a transparent yellow azo dye image.

## Example III

In experiments similar to those described under Example I, the phenylhydrazine is replaced by an equal amount of o-, m- or p-tolylhydrazine. The resulting films are similar in appearance to those described in Example I. The azo dyes have the following probable structure:



Example IV

In experiments similar to those described under Example II, the phenylhydrazine was replaced by o-, m- or p-tolylhydrazine. The resulting films are similar in appearance to those described in Example II. The azo dyes have the following probable structure:



Example V

In an experiment similar to those described in Examples I, the phenylhydrazine is replaced by 10 cc. of p-nitrophenylhydrazine hydrochloride solution containing 1.5 parts per 100 parts of water. The resulting films contain bright red azo dye images. The dye has the following probable structure:



Example VI

In experiments similar to those described in Example II, the phenylhydrazine is replaced by p-nitrophenylhydrazine hydrochloride solution as in Example V. The resulting films contain bright orange-yellow azo dye images. The dye has the following probable structure:



Example VII

A developing solution is prepared by dissolving 0.5 part of p-nitrophenylhydrazine hydrochloride

in 90 parts of water to which is added 8 parts of 2% sodium oleate solution, 5 grams of sodium acetate, 1 part of acetic acid and 1 part of 1-dimethylamino-5-naphthol. This developing solution is used in experiments similar to those described in Example I. The resulting films contain transparent images of blue azo dyes of the following probable structure:



Example VII

15

16

17

18

19

20

21

22

23

24

25

26

27

28

29

30

31

32

33

34

35

36

37

38

39

40

41

42

43

44

45

46

47

48

49

50

51

52

53

54

55

56

57

58

59

60

61

62

63

64

65

66

67

68

69

70

71

72

73

74

75

76

77

78

79

80

81

82

83

84

85

86

87

88

89

90

91

92

93

94

95

96

97

98

99

100

101

102

103

104

105

106

107

108

109

110

111

112

113

114

115

116

117

118

119

120

121

122

123

124

125

126

127

128

129

130

131

132

133

134

135

136

137

138

139

140

141

142

143

144

145

146

147

148

149

150

151

152

153

154

155

156

157

158

159

160

161

162

163

164

165

166

167

168

169

170

171

172

173

174

175

176

177

178

179

180

181

182

183

184

185

186

187

188

189

190

191

192

193

194

195

196

197

198

199

200

201

202

203

204

205

206

207

208

209

210

211

212

213

214

215

216

217

218

219

220

221

222

223

224

225

226

227

228

229

230

231

232

233

234

235

236

237

238

239

240

241

242

243

244

245

246

247

248

249

250

251

252

253

254

255

256

257

258

259

260

261

262

26

5-pyrazolone. The resulting films contained bright yellow azo dye images. These dyes have the following probable structures:



Example XIV

In a series of experiments similar to those described under Examples I, III and V, the sodium  $\beta$ -naphtholate was replaced by 2,4-dihydroxy-quinoline. The resulting films contained yellow azo dye images. These dyes have the following probable structure:



Example XV

A photographic emulsion containing silver halide and stearoyl-J-acid in the ratio of 10 to 1 was coated on a cellulose acetate base, exposed and developed in a non-color-forming developer such as Metol-hydroquinone, then re-exposed and processed in a solution made as follows: Two parts of phenylhydrazine is dissolved in a mixture of 90 parts of water and 8 parts of 2% sodium oleate solution, and to this is added 2 grams of sodium carbonate. After development for 15 minutes at 8° C., the film is washed, the silver bleached as in potassium ferricyanide solution and the silver salts removed with sodium thiosulfate. The resulting film contains a bright orange-red azo dyestuff image. This dye has the following probable structure:



Example XVI

In experiments similar to that described under Example XV, the phenylhydrazine is replaced by o-, m-, or p-tolylhydrazine in equal amounts. The resulting films appear similar to those described under Example XV. The azo dyes have the following probable structure:



Example XVII

In experiments similar to that described under Example XV, the phenylhydrazine is replaced by p-bromo-phenylhydrazine in equal amounts. The resulting films appear similar to those produced in Example XV, and the azo dye has the following probable structure:



Example XVIII

In experiments similar to that described under Example XV, the phenylhydrazine was replaced by an equal amount of p-nitrophenylhydrazine. 5 The resulting film contained bright magenta dye images. This dye has the following probable structure:



Example XIX

In experiments similar to that described under Example XV, the phenylhydrazine was replaced by p-hydrazino-diphenyl. The resulting films 15 contained magenta dye images. This dye has the following probable structure:



Example XX

A photographic emulsion containing 1 part of p-dodecylacetanilide to 10 parts of silver halide is coated on cellulose acetate film base and treated as the films in Examples XV to XIX, inclusive. The films all contained yellow to orange azo dyes. These dyes have the following probable structure:



In place of the films used in any of the preceding examples, it is possible to use films prepared by removing the silver image, after the first development, with a reversal bath such as one containing chromic acid or sulfuric acid and a dichromate, and the like, and then reducing the remaining silver salts and reoxidizing them with a ferricyanide, an acid chromate, or a copper halide, to silver salts which are more readily reducible by the hydrazines. Similarly, if the films used in any of the preceding examples are exposed to light through films bearing negative images, they may be developed in a Metol-hydroquinone developer, and then fixed and the silver reoxidized according to the method of the preceding sentence and then color developed as described in the preceding examples to yield images in azo dyes.

Example XXI

To a mixture of 90 parts of water and 5 parts of 2% sodium oleate solution is added 2 parts of phenylhydrazine, 2 parts of sodium carbonate, and 1 part of sodium beta-naphtholate. A photographic film containing a light-sensitive silver-halide-gelatin emulsion layer is exposed and developed in this bath at 8° C. The development 65 requires about ten to fifteen minutes. After development the film is thoroughly washed and placed in a 4% solution of potassium ferricyanide for five minutes, washed, and placed in 25% sodium thiosulfate for five minutes, then thoroughly washed. The resulting film contains a

clear bright orange azo dye image. The dye has the following probable structure:



The reduction of silver salts by aromatic amino compounds is believed to proceed with oxidation of the amine group to a nitroso group or a group readily convertible to the same, for in the development of silver salts with p-aminodiethylaniline in the presence of phenol an indoaniline dye is produced the structure of which indicates that it is derived from p-nitrosodiethylaniline and phenol. In the case of phenylhydrazine, if the reaction proceeds in the same manner, the product might be expected to be phenylnitrosoamine. The aromatic nitrosoamines are known to be in tautomeric equilibrium with the diazo compounds, which will couple with aromatic phenols, amines and active methylene compounds to produce azo dyes. That the reaction occurs in some such manner as this seems likely, since development of silver salts with phenylhydrazine in the presence of beta-naphthol yields the same azo dye as produced from the benzene diazonium compound and beta-naphthol.

In place of the specific aromatic hydrazines of each of the respective examples may be substituted other aromatic hydrazines which have developing powers and are capable of reducing silver salts to metallic silver. Suitable reducing or developer baths are described in U. S. P. 2,220,929. Among the useful primary aromatic hydrazines are

Tolylhydrazines  
Nitrophenylhydrazines  
Bromophenylhydrazines  
Chlorophenylhydrazines  
Chloronaphthylhydrazines  
Bromonaphthylhydrazines  
p-Diphenylhydrazines  
p,p'-Diphenyldihydrazines  
Alpha-naphthylhydrazines  
Beta-naphthylhydrazines

A small amount of a mild oxidizing agent may be used in each of the developing processes described above. In general amounts up to 2% give satisfactory results. Suitable oxidizing agents in addition to those recited above include alkali metal peroxides, perborates, percarbonates, alkali metal salts of perorganic acids, e. g. peracetic acid, perpropionic acid, etc.

The invention is not limited to the treatment of ferrocyanide bleached images; on the contrary silver salt images such as silver chloride, silver bromide, silver chloro-bromide, silver iodide, silver ferricyanide, and the complex silver copper salts may be used.

The invention is not limited to the non-migratory coupling components above described, but other coupling components which, on account of their chemical constitution or molecular size, remain firmly bound in gelatin films, for example, and are not leached from them nor migrate in them when the films are placed in the customary baths used in color photography. Many compounds of this type are described in the literature. Suitable compounds are set forth in British Patents 458,400, 465,823, 479,838, 489,161, 76

489,274, 489,093, 483,000 and French Patents 830,878 and 830,926.

The color development procedures hereof are, furthermore, not limited to any specific type of photographic element. Thus, they are applicable to photographic films and plates bearing a single emulsion layer or to multilayer photographic elements. Thus, mono-, bi- and tri-packs may be processed. In the case of such multilayer films 10 and plates, the azo coupling components are chosen so that they form dyes upon treatment with the hydrazine reducing baths hereof, which dyes are complementary in color to the utilized sensitivity range of the respective emulsion layer 15 in which they are incorporated. Upon exposure to a natural color scene, such films can be developed in a non-color-forming developer and, without removing the thus formed silver images or re-exposing, the residual silver salts can be reduced with one of the hydrazine solutions hereof. Upon removal of all of the silver images, a positive transparency in natural colors is formed.

The invention is also useful with stripping films whereby the emulsion layers are releasably 20 attached to a photographic element support which may be paper or a cellulosic ester or ether film base or a resin. The sensitive emulsion of such films is coated onto a thin menstruum of collodion which in turn has been coated onto a water soluble adhesive layer such as glue or dextrine which in its turn has been coated onto a suitably prepared temporary support of the type previously described. The adhesive layers may be of the type which is softened or dissolved in 30 water, alkaline baths, e. g. developer baths or acid baths and reversal bleach baths. Various types of stripping photographic elements useful in accordance with this invention are described in Marasco application, Serial No. 245,274, filed 40 December 12, 1938 now U. S. P. 2,182,814.

Color separation negatives may be printed onto a stripping paper stock. The negative thus printed is fixed in bleached, washed and redeveloped in the hydrazine developers hereof containing the proper and desired coupling component. The color development processes hereof constitute a distinct advance to this art because the previously available toning methods lack 50 brilliancy and the transparency of dye images.

This invention has the advantage that, while the processing of the films is fully as simple as in the previously discovered processes of color development, the colors produced are more stable. Azo dyes as a class are known to be much more 55 stable than those used in the other processes, and it is possible to obtain a much wider range of colors, thus approximating more nearly the ideal colors for a perfect three-color subtractive process. This process then has all of the advantages of the former process without many of its disadvantages such as short life of the film and failure to reproduce natural colors faithfully.

As many apparently widely different embodiments of this invention may be made without departing from the spirit and scope thereof, it is to be understood that I do not intend to limit myself to the specific embodiments herein except as defined by the appended claims.

We claim:

- 70 1. In a photographic reversal process the step of developing the reversed silver salt image in a developing solution containing as the sole type of reducing agent an aromatic hydrazine, in the presence of an azo coupling component.
2. In a photographic reversal process compris-

ing exposure of a photographic element containing silver salts to an image, development in a non-color forming photographic developer, re-exposure to light and re-development, the step of developing the reversed image in a developing solution containing as the sole type of reducing agent an aromatic hydrazine, in the presence of an azo coupling component.

3. The method of producing a direct positive by a reversal process which comprises exposing an emulsion layer containing light sensitive silver salts, developing said layer in a non-color-forming photographic developer and reducing the residual image in a developing solution containing as the sole type of reducing agent an aromatic hydrazine, in the presence of an azo coupling component, and removing the silver images.

4. The process which comprises developing a bleached silver salt image in a developing solution containing as the sole type of reducing agent an aromatic hydrazine, in the presence of a coupling component to form a dye.

5. The process which comprises developing a bleached silver salt image in a developing solution containing as the sole type of reducing agent an aromatic hydrazine, in the presence of an azo coupling component to form an azo dye image.

6. A process which comprises developing a photographic element having at least one layer containing reducible silver salts in a developing solution containing as the sole type of reducing agent an aromatic hydrazine, in the presence of a mild oxidizing agent and a coupling component to form a dye.

7. A process which comprises developing a photographic element containing a silver salt image in a developing solution containing as the sole type of reducing agent an aromatic hydrazine, in the presence of a mild oxidizing agent and an azo coupling component to form an azo dye image.

8. An aqueous alkaline developer solution containing a mild oxidizing agent, an azo dye coupling component and as the sole type of reducing agent a primary aromatic hydrazine characterized by its ability to precipitate silver from an ammoniacal solution containing approximately 0.1% of silver nitrate in 30 seconds at 20° C.

9. A process which comprises developing a photographic element having at least one layer containing reducible silver salts in a developing solution containing as the sole type of organic reducing agent a primary aromatic hydrazine characterized by its ability to precipitate silver from an ammoniacal solution containing approximately 0.1% of silver nitrate in 30 seconds at 20° C. in the presence of an azo coupling component to form a dye.

10. A process which comprises developing a photographic element containing a silver salt image in a developing solution containing as the sole type of organic reducing agent a primary aromatic hydrazine characterized by its ability to precipitate silver from an ammoniacal solution containing approximately 0.1% of silver nitrate in 30 seconds at 20° C. in the presence of an azo coupling component to form a dye.

11. In a photographic reversal process the step of developing the reversed silver salt image in a developing solution containing as the sole type of organic reducing agent a primary aromatic hydrazine characterized by its ability to precipitate silver from an ammoniacal solution containing approximately 0.1% of silver nitrate in 30 seconds at 20° C. in the presence of an azo coupling component to form a dye image.

12. A process which comprises developing a silver ferrocyanide image in a developing solution containing as the sole type of organic reducing agent an aromatic hydrazine in the presence of an azo coupling component to form an azo dye image.

13. The method of producing a direct positive by a reversal process which comprises exposing a photographic element bearing an emulsion layer containing light sensitive silver salts and a non-migratory azo coupling component, developing said layer in a non-color forming photographic developer and reducing the residual silver salt image in a developing solution containing as the sole type of organic reducing agent an aromatic hydrazine, and removing the silver and silver salts.

14. A process which comprises developing a photographic element containing a silver salt image in an aqueous developer solution containing as the sole type of reducing agent an aromatic hydrazine dissolved in an aqueous solution containing not more than 1% of a long chain surface active polar compound containing a hydrophilic group and a hydrophobic group of at least 8 carbon atoms in the presence of a coupling component to form a dye.

15. A process which comprises developing a photographic element containing a silver salt image in a developing solution containing as the sole type of reducing agent monophenylhydrazine and an azo coupling component containing a phenolic group to form an azo dye image.

16. A process which comprises developing a photographic element containing a silver salt image in a developing solution containing as the sole type of reducing agent para-nitrophenyl hydrazine and an azo coupling component containing a reactive methylene group to form an azo dye image.

17. A process which comprises developing a photographic element containing a silver salt image in a developing solution containing as the sole type of reducing agent para, para'-diphenyldihydrazine and an azo coupling component, containing aromatic amino groups to form a dye image.

18. A process which comprises developing a photographic element containing a silver salt image in a developing solution containing as the sole type of reducing agent an aromatic hydrazine dissolved in an aqueous solution containing not more than 1% of sodium oleate in the presence of an azo coupling component to form an azo dye image.

DAVID W. WOODWARD.  
DAVID M. McQUEEN.